

Aug. 26, 1924.

1,506,053

C. G. FINK

METALLURGY OF TIN

Filed March 17, 1921



Colin G. Fink Inventor

By his Attorneys

Perkins, Davis, Nease & Edmunds

## UNITED STATES PATENT OFFICE.

COLIN G. FINK, OF YONKERS, NEW YORK, ASSIGNOR TO GUGGENHEIM BROTHERS,  
A COPARTNERSHIP, OF NEW YORK, N. Y.

## METALLURGY OF TIN.

Application filed March 17, 1921. Serial No. 452,951.

To all whom it may concern:

Be it known that I, COLIN G. FINK, a citizen of the United States, residing at Yonkers, in the county of Westchester, State of New York, have invented certain new and useful Improvements in the Metallurgy of Tin; and I do hereby declare the following to be a full, clear, and exact description of the invention, such as will enable others skilled in the art to which it appertains to make and use the same.

This invention relates to metallurgical processes for the recovery of tin from tin-containing materials. More particularly, the invention relates to the recovery of tin from tin oxide ores, such as native or roasted tin ores or concentrates, or other appropriate tin-containing materials. The invention has for its object the provision of certain improvements in the metallurgy of tin, and, in particular, contemplates the provision of an improved method of recovering tin from appropriate tin-containing materials.

It has heretofore been the general practice in tin metallurgy to smelt tin ores, or other appropriate tin-containing materials in a reverberatory or shaft furnace employing a solid carbonaceous material, such as coke, as the reducing agent. In these heretofore customary processes, the reduction of the tin compounds is brought about by carbon monoxide gas produced by the union of the carbonaceous material of the charge with air blown into or otherwise appropriately brought into contact with the charge. The formation of carbon monoxide by the reaction between solid carbonaceous material, such as coke, and air, does not readily take place at temperatures below about 1100° C., and it is therefore necessary in smelting tin compounds with solid carbonaceous material to heat the charge to a temperature above 1100° C. in order to effect the necessary formation of carbon monoxide gas for the reduction of the tin compounds. Thus, in the heretofore customary reverberatory furnace practice, the charge, consisting, for example, of a native oxide or a roasted tin ore and coke and generally an appropriate fluxing agent, is brought to a temperature above 1100° C. so as to form, by the combustion of the coke, the carbon monoxide gas required for the reduction of the tin compounds to metallic tin. Substantially the same metallurgical reactions are

involved in the smelting of tin-containing materials in accordance with the heretofore customary shaft furnace practice. However, it is usually the practice in smelting tin ores in a shaft furnace to supply the charge in alternate layers of coke and ore, in order to provide, by the combustion of the layers of coke and ore, in order to provide, by the combustion of the layers of coke as they progressively reach the active combustion zone of the furnace, a sufficiently high temperature to effect the production of carbon monoxide gas for the reduction of the tin compounds in the superposed layer of ore. In both the reverberatory and shaft furnace practice, it has heretofore been customary to include in the charge an appropriate fluxing agent, such as limestone, and two molten products, (1) reduced metallic tin and (2) slag, are appropriately withdrawn from the furnace.

The higher oxide of tin, unlike the higher oxides of copper and lead, is not readily dissociated by heat into the lower oxide. For example, in the smelting of copper and lead ores heat alone reduces the higher oxides of copper or lead ( $CuO$  or  $PbO_2$ ) to lower oxides of copper or lead ( $Cu_2O$  or  $PbO$ ). As a result of this dissociation of the higher oxides into the lower oxides and oxygen by heat alone, oxygen is liberated within the charge itself, being in fact generated in situ, and this liberated oxygen combines with the carbonaceous material of the charge and forms carbon monoxide which effectively assists in the smelting operation. The oxygen thus liberated by the action of heat alone is more or less diffused throughout the body of the charge and insures, to a certain extent, the presence of a considerable amount of oxygen within the charge itself. On this account, it is not difficult in copper and lead smelting to effect a satisfactory diffusion within the body of the charge of sufficient oxygen for smelting purposes, since the charge is kept porous by the liberated oxygen and carbon monoxide and the externally derived air blown into or otherwise appropriately brought into contact with the charge is effectively augmented by the oxygen liberated within the charge itself by the dissociation of the higher metal oxides into lower oxides and oxygen by the action of heat alone.

In the smelting of tin ores, on the other

hand, the natural diffusion of oxygen throughout the charge itself cannot be relied upon, because the higher oxide of tin ( $\text{SnO}_2$ ) is not readily dissociated by heat alone into the lower oxide ( $\text{SnO}$ ) and oxygen, and at the temperatures usually prevailing in the heretofore customary processes of tin smelting this dissociation does not take place to any appreciable extent.

5 For this reason, in the smelting of tin ores in the reverberatory furnace, the charge is not permeated to any appreciable extent with oxygen liberated from the compounds of tin by the action of heat alone. It is

10 very important for the satisfactory smelting of tin ores that effective measures be employed to insure the necessary contact of the carbonaceous material of the charge with externally derived air for effecting the

15 formation of the carbon monoxide gas required for the reduction of the tin compounds. In the reverberatory smelting of tin ores, practically only the surface of the charge receives sufficient oxygen for the

20 combustion of the carbonaceous material, and for this reason it is necessary to constantly rabble or work the charge in order to bring fresh material to the surface where the effective reaction is taking place. Moreover, at the relatively high temperature at

25 which coke and air readily react to form carbon monoxide, namely, at temperatures of about  $1100^\circ \text{ C.}$ , there is a tendency in tin smelting for the charge to fuse before the tin compounds therein have been properly reduced, thereby rendering the surface of the charge still less pervious to the diffusion of gases and more effectively confining the reduction to the surface.

30 In the smelting of tin ores in shaft furnaces, in accordance with the heretofore customary practice, substantially the same objectionable conditions are encountered as in reverberatory smelting. The high temperature required for the formation of carbon monoxide tends to fuse the ore before the tin compounds therein have been properly reduced, thus rendering the ore less pervious to the effective diffusion of the carbon

35 monoxide gas. Thus, in both the heretofore customary reverberatory and shaft furnace smelting of tin ores, the first slag generally contains from 20% to 40% of tin due to the inability of the carbon monoxide gas to effectively reach all parts of the metalliferous material in the charge as well as to the great tendency of tin to combine with the gangue and the fluxing agents in the charge at the relatively high temperature

40 necessarily employed.

The method of the present invention involves a radical departure from the heretofore customary processes of smelting tin ores. Thus, in accordance with the present invention, the tin-containing material is

45 first subjected to a reducing treatment in the course of which the compounds of tin are reduced to metallic tin by a gaseous reducing agent without fusion of the non-metallic or gangue constituents of the material and, if desired, without material agglomeration of the reduced metal. The product of this reducing treatment is a mixture in which the reduced tin is more or less scattered throughout the non-metallic

50 constituents of the original ore, and the next step in the method of the invention consists in effecting the separation of the metallic tin from the aforementioned mixture. This separating step may be carried out in various ways, as will be fully described hereinafter. The aforementioned reducing treatment may be considered in the nature of a preparatory step for the subsequent separation of the metallic tin from the

55 gangue constituents of the ore, and as a result of this reducing or preparatory treatment, there is obtained a mixture of metallic tin and gangue from which the metallic tin can be subsequently separated by various

60 satisfactory procedures.

I have found that externally prepared gaseous reducing agents, such as hydrogen, carbon monoxide, or the like, effectively reduce stannic oxide to metallic tin at temperatures in the neighborhood of  $550^\circ \text{ C.}$  to  $900^\circ \text{ C.}$  At these relatively low temperatures fusion of the charge does not take place and the charge remains extremely permeable to the gaseous reducing agent. Moreover, these relatively low temperatures are well above the melting temperature of metallic tin. Thus, in accordance with my present invention, the tin-containing material is heated to a temperature relatively low as compared with the heretofore customary practice in tin-smelting and a gaseous reducing agent is then blown into or otherwise appropriately brought into contact with the heated charge. Preferably, no fluxing agents are mixed with the charge, and the reducing operation merely involves heating the tin-containing material, for example, roasted tin ore or concentrates, to a temperature of from  $550^\circ \text{ C.}$  to  $900^\circ \text{ C.}$  and subjecting the thus heated material to the action of a gaseous reducing agent, such as hydrogen, carbon monoxide, or a mixture thereof, the reducing agent being introduced into the charge in gaseous form.

In the practice of the invention, the tin ore, concentrate, or the like, preferably in a finely divided condition, is heated to a temperature of from  $550^\circ \text{ C.}$  to  $900^\circ \text{ C.}$ , for example, by a gas furnace or by electrical means. The heating or reducing chamber may advantageously take the form of a slightly inclined tube or chamber adapted to have the ore fed in at one end and the products of the reaction discharged at the

other end, and provided with means for the supply thereto of hydrogen or other appropriate gaseous reducing agent, and the removal therefrom of the exhaust gases. 5 Where the inclination of the reaction chamber is not sufficient to insure the passage of the ore through the tube or chamber by gravity, suitable conveying or rabbelling means may be provided, or the tube or chamber may be rotated to insure agitation 10 of the charge and uniform treatment thereof, together with gradual progression of the charge through the reaction chamber.

The portions of the reaction chamber contacting with or exposed to the charge during the reaction should be made of a material adapted to withstand the corrosive effects characteristic of the reaction. Thus, the reaction chamber may be made of or 15 lined with suitable refractory material, such, for example, as an iron tube or cylinder lined with magnesite. I prefer, however, to employ a tube or chamber composed of, or appropriately lined with, an alloy of iron 20 and chromium containing not less than about 30% of chromium. I have secured satisfactory results with ferro chromium alloys containing from 30% to 60% of chromium. Alloys of iron with other metals 25 may also be used in making or lining the reaction chamber. For example, titanium, uranium, vanadium and manganese form with iron suitable alloys for the reaction chamber. The above named metals possess 30 the common property that their oxides are not completely reduced by hydrogen at the reaction temperature characteristic of the invention.

The tin ore or concentrate is heated in the reaction chamber or furnace to a suitable temperature, temperatures between 550° C. and 900° C. being satisfactory, and hydrogen or other appropriate gaseous reducing agent, is brought into contact therewith in 5 a sufficient amount and for a sufficient period of time to insure reduction of the tin oxide. The selection of the best reducing temperature is of great importance for efficient operation. It is well known that 10 as a general rule the velocity of a chemical reaction increases rapidly with the temperature. Accordingly, as far as the chemical reduction of tin oxide is concerned high temperatures, of 1000° C. and over, are to 15 be preferred. However, aside from the fume losses at high temperatures, I find that it is good practice to keep the charge porous and prevent fusion or slagging. For, as is pointed out herein, the quantity of tin 20 concentrates reduced per unit of time is dependent not directly upon the chemical reaction velocity but upon the diffusion velocity of the reducing gas and water vapor produced. It is readily appreciated that a 25 reducing gas such as hydrogen will pass

through a porous charge more rapidly than through a fused charge. Accordingly, a temperature as little below the slagging point of the gangue as possible should be selected in order to secure the best results. 70 This slagging point varies from one lot of concentrates to the other, depending largely upon the relative amounts of silica, iron, lime, etc., in the gangue. Tin concentrates rich in tourmaline usually have a low slagging point; the addition of a little lime 75 will raise this point.

The reduction takes place without difficulty and results in the production of metallic tin more or less scattered throughout the finely divided gangue or non-metallic constituents of the original ore. At temperatures around 650° C. and higher, the reduced metallic tin tends to run together or agglomerate, and may, under appropriate 80 operating conditions, be withdrawn from the furnace in a liquid metallic state. At lower temperatures, the reduced metallic tin remains more or less distributed throughout the charge in admixture with the gangue etc. The reduced metallic tin may, accordingly, be distributed throughout the work-off charge in a finely divided state, or may be somewhat agglomerated and more or less porous, or may, to a greater or less extent, 85 be recovered from the furnace in a liquid metallic state and directly cast or solidified in ingots or in the form of anodes for use in electrolytic refining. No particular precautions appear necessary at the end of the 90 reducing treatment to prevent reoxidation of the metallic tin.

Where the tin is in part agglomerated together in the product discharged from the furnace, this product may be appropriately treated to remove or separate the gangue, to the desired extent, from the reduced tin. This separation may be brought about by heating the mixture of reduced metallic tin and gangue to temperatures of 1000° C. to 105 1200° C., with or without the addition of fluxes. This heating may be carried out in any appropriate type of furnace, such, for example, as a crucible furnace, and the metallic tin will melt and collect in the bottom 110 of the furnace or crucible and may be appropriately withdrawn therefrom and thus separated from the gangue originally admixed therewith. The separation of the gangue from the reduced metallic tin may 115 also be effected by subjecting the mixed product of the reducing treatment to a grinding and hydraulic classifying operation or to other appropriate concentrating or classifying treatments. The desired separation of the reduced metallic tin from the gangue in the worked-off charge may 120 furthermore be advantageously effected by centrifugal action in the course of which the worked-off charge, heated to a sufficiently 125 130

high temperature to melt the reduced metallic tin, is centrifuged in an appropriate centrifugal apparatus, preferably heated to maintain the metallic tin in a liquid or 5 melted condition, whereby the melted tin is discharged from the apparatus by centrifugal action.

The most effective gaseous reducing agent for the practice of the invention is hydrogen. Hydrogen gas for the purpose of the 10 invention may be obtained from any suitable source, for example, electrolytic hydrogen may be advantageously employed. Many gases containing hydrogen, carbon 15 monoxide, or hydrocarbons, or containing two or all of said gaseous reagents, may be employed in the practice of the invention, and I merely mention by way of example, water gas, producer gas, illuminating gas, 20 oil gas and hydrocarbon vapor or vapors as appropriate gaseous reducing agents for the practice of the invention. It will be understood by those skilled in the art that various hydrocarbon and similar compounds which 25 are decomposed at the reaction temperature contemplated by the invention into volatile reducing agents may be employed as the source of the gaseous reducing agents for the purposes of the invention. Thus, methane, benzine, alcohol and the like may 30 serve as the source of an appropriate gaseous reducing agent for the purposes of the invention.

When using ores containing metallic sulfides it is advantageous, though not absolutely essential, first to roast the ore so as to convert the metallic sulfides to metallic oxides, and then to subject the roasted ore, while still hot from the roasting treatment, 35 to reduction with hydrogen or other appropriate gaseous reducing agent, thereby economizing in the amount of heat required, and taking advantage of the hot reactive condition of the freshly roasted ore. The roasting operation may be effected in the same 40 furnace in which the ore is to be subsequently reduced, or in a separate furnace from which the roasted ore is directly discharged into the reducing furnace. The feed of the 45 ore to the reducing furnace may be continuous where the furnace is provided with means for the continuous supply thereto of ore and the continuous discharge therefrom of the worked-off charge, or the feed to the 50 reducing furnace may be intermittent and successive charges of ore subjected therein to the reducing treatment.

Any sulfur occurring in small amounts in native or raw oxide or oxidized ores, or any 55 unoxidized sulfur remaining in a roasted sulfide ore, will be subjected to the reducing action of the hydrogen during the reduction of the ore, with the resulting formation of hydrogen-sulfide. The addition of small 60 amounts of chlorine or hydrochloric acid,

for example, by mixing chlorine gas or hydrochloric acid gas with the hydrogen gas or by otherwise adding chlorine or hydrochloric acid to the ore, accelerates the removal of sulfur.

I prefer, in practicing the present invention, to add no fluxing agent to the charge. By the improved process of the invention, the compounds of tin are reduced, at relatively low temperatures as compared with 70 prior processes of tin smelting, without necessitating the fusion or slagging of the gangue constituents in the ore. In fact, one of the peculiar advantages of the process of the invention resides in the fact that only 75 the reduced metallic tin is melted at the prevailing reaction temperatures, and the gangue material in the ore remains solid throughout the entire reducing operation. When smelting tin ores of comparatively 80 low melting point, for example, ores containing large percentages of tourmaline, lime-stone (2%-10%) may be added to the ore to counteract any tendency which the 85 gangue of the ore may display to fuse or melt.

As hereinbefore mentioned, the method of the invention may advantageously be carried out as a continuous process, by supplying the ore to the furnace in a continuous or 90 intermittent manner and similarly withdrawing the reduced tin and ore residue and by supplying the hydrogen, or other appropriate reducing gas, in a continuous and regulable manner. The gaseous reducing 95 agent may advantageously be introduced near the discharge end of the furnace so that it comes in contact first with the reduced and partly reduced ore, thus insuring complete reduction. By proper supply and 100 regulation of the supply of the gaseous reducing agent, substantially complete utilization of the reducing gas can be secured so that the gases discharged from the furnace 105 will be made up of steam, carbon dioxide, and inert gases.

I prefer, however, to use an excess of hydrogen or other suitable reducing gas and to keep this gas in constant circulation allowing it to sweep over the charge at a comparatively rapid rate for example 40 cu. ft. per square foot of hearth per hour. As the gas leaves the furnace and before reentering it, the products of combustion, such as water, 110 are preferably removed. I have found that the velocity of reduction is largely dependent upon the speed with which the water vapor (in the case of reduction by hydrogen) is removed. The velocity of reduction is proportional to the speed of the diffusion of the reducing gas through a film of water covering the tin oxide particles. The chemical reaction between the tin oxide and hydrogen is comparatively rapid at temperatures of 600° C. and above.

A suitable apparatus for use in carrying out the invention is illustrated in the accompanying drawing in which the figure illustrates a sectional view of a furnace and crucible in which the material may be treated.

Referring to the drawing, 5 indicates the brick-work forming the support for the furnace tube 6 which may be constructed of any suitable material as hereinbefore suggested, but which is preferably made from an alloy of iron and chromium containing not less than about 30% of chromium. The furnace tube may be heated by any suitable means, 10 the electric heating element 7 being shown by way of illustration. The finely divided material is supplied to the furnace tube through an inlet 8, and its movement through the tube is facilitated by a rabble 9 which is 15 also constructed preferably of the iron chromium alloy. The rabble 9 is supported on a shaft 10 carried in suitable bearings at the ends of the tube and driven through a gear 11 or the equivalent driving connection 20 from a source of power.

The reducing gas, such as hydrogen, is supplied to the furnace tube through a pipe 12 connected to a source of supply, and as the hydrogen passes through the mass of 25 material under treatment the reducing action hereinbefore described is carried on for the accomplishment of the intended purpose. The operation of the furnace may be such that reduced material is continuously 30 or intermittently withdrawn therefrom, and this material may be delivered into a crucible 13 which is preferably heated by an electric arc between electrodes 14 and 15, the latter being supplied with power through 35 cables 16. Preferably a pipe 17 permits the introduction of a reducing gas such as hydrogen to the crucible to prevent oxidation of the contents. In the crucible the reduced 40 tin separates and descends to the bottom 45 from which it may be withdrawn through a tap 18. The overlying slag may be withdrawn similarly through a tap 19.

The details of the structure described are 50 merely illustrative of a possible form of apparatus. These details may be varied, and other means may be substituted for the furnace tube and crucible as hereinbefore set forth.

The reduced metallic tin, whether in a 55 solid metallic state or admixed with the gangue constituents of the ore, is well adapted for electrolytic refining. When the tin runs out of the furnace as metallic tin, this 60 may be cast in the form of anodes and these anodes used in the electrolytic refining operation. Where the reduction is carried out at relatively low temperatures, so that the reduction product is porous, this product can 65 be compressed and used in the electrolytic refining process without preliminary separa-

tion of the reduced tin from the gangue, or the reduction product can be concentrated and the concentrate compressed and used as the anode in the electrolytic process. Tin thus produced is well adapted for electrolytic 70 refining by the process of my application for Letters Patent of the United States, Serial No. 533,249; filed February 1, 1922 making use of an electrolyte containing a preponderating concentration of sulfate ions with 75 respect to other anions present therein and a preponderating concentration of ions of a metal more electropositive than tin with respect to other cations present in the electrolyte. 80

I claim:—

1. A metallurgical process for the treatment of tin ores, concentrates, or other appropriate tin-containing material, which comprises heating the tin-containing material to an elevated temperature but below the fusing temperature of the non-metallic constituents of the charge, and bringing an externally prepared gaseous reducing agent 85 into intimate contact with the thus-heated material and thereby reducing the compounds of tin to metallic tin without fusion of the non-metallic constituents of said material. 90

2. A metallurgical process for the treatment of tin ores, concentrates or other appropriate tin-containing material, which comprises heating the tin-containing material to a temperature of from 550° C. to 900° 95 C., and bringing an externally prepared gaseous reducing agent into intimate contact with the thus-heated material and thereby reducing the compounds of tin to metallic tin without fusion of the non-metallic constituents of said material. 100

3. A metallurgical process for the treatment of tin ores, concentrates or other appropriate tin-containing material, which comprises heating the tin-containing material to a temperature of from 500° C. to 900° 110 C., and bringing a gaseous reducing agent containing hydrogen gas and carbon monoxide gas into intimate contact with the thus-heated material and thereby reducing the compounds of tin to metallic tin without fusion of the non-metallic constituents of said material. 115

4. A metallurgical process for the treatment of tin ores, concentrates or other appropriate tin-containing material, which comprises heating the tin-containing material to a temperature of from 550° C. to 900° C., and bringing hydrogen gas into 120 intimate contact with the thus-heated material and thereby reducing the compounds of tin to metallic tin without fusion of the non-metallic constituents of said material. 125

5. A metallurgical process for the treatment of tin ores, concentrates, or other appropriate tin-containing material, which 130

comprises heating the tin-containing material, which comprises heating the tin-containing material to an elevated temperature but below the fusing temperature of 5 the non-metallic constituents of the charge, bringing an externally prepared gaseous reducing agent into intimate contact with the thus-heated material and thereby reducing the compounds of tin to metallic tin with- 10 out fusion of the non-metallic constituents of said material and producing a product in which the reduced metallic tin is more or less scattered throughout said non-metallic constituents, and subjecting 15 said product to appropriate subsequent treatment for the segregation and separation therefrom of the metallic tin.

6. A metallurgical process for the treatment of tin ores, concentrates, or other appropriate tin-containing material, which comprises heating the tin-containing material in a finely divided condition to a temperature of from 550° C. to 900° C., bringing an externally prepared gaseous reducing agent into intimate contact with the thus-heated material and thereby reducing the compounds of tin to metallic tin with- 20 out fusion of the non-metallic constituents of said material and producing a product of finely divided physical condition in which the reduced metallic tin is more or less scattered throughout said non-metallic constituents, and subjecting said product to appropriate subsequent treatment for the 25

segregation and separation therefrom of the 30 metallic tin.

7. A metallurgical process for the treatment of tin ores, concentrates, or other appropriate tin-containing material, which comprises subjecting the material to the 40 action of a gaseous reducing agent together with a small amount of chlorine or hydrochloric acid at a temperature of from 550° C. to 900° C.

8. The method of recovering tin from sulfide ores, which comprises roasting the ore, and subjecting the roasted ore to the action of hydrogen at an elevated temperature, small amounts of chlorine or hydrochloric acid being added to promote the removal 45 of any remaining sulfur.

9. The method of recovering tin from oxidized ores or concentrates containing sulfur, which comprises subjecting the ore to the action of hydrogen and small amounts 50 of chlorine or hydrochloric acid at a temperature of about 600° to 850° C.

10. The method of recovering tin from oxidized ores, concentrates, or other appropriate tin-containing material, which comprises subjecting the tin-containing material to the action of hydrogen at an elevated temperature, and separating the reduced tin from the resulting product by centrifugal action at a sufficiently high temperature to 55 melt the tin.

In testimony whereof I affix my signature.  
COLIN G. FINK.